

# UNITED STATES PATENT OFFICE.

JOHN BARRINGTON, OF BOSTON, MASSACHUSETTS.

## ALKALI-FREE DETERGENT FOR SCOURING AND DYEING AND PROCESS OF MAKING SAME.

1,139,326.

Specification of Letters Patent. Patented May 11, 1915.

No Drawing.

Application filed June 2, 1914. Serial No. 842,464.

To all whom it may concern:

Be it known that I, JOHN BARRINGTON, a citizen of the United States, residing in the city of Boston, county of Suffolk, State of Massachusetts, have invented a new and useful Alkali-Free Detergent for Scouring and Dyeing and Process of Making Same, of which the following is a specification.

My invention relates to a new and useful detergent or soap dye, method of producing, and process for employing the same, the detergent consisting of a neutral vegetable oil soap, sulfonated castor oil, and an anilin color in suitable proportions, and in the method of employing the same, in adding a neutral product which is capable of forcing the dye out of the boiling dye bath, and on the material, both animal and vegetable fibers, which will color same thoroughly and permanently.

My new compound consists of a mixture containing a neutral vegetable oil soap, such as neutral cocoanut oil soap, sulfonated castor oil, and an anilin color or colors, which may be of the color desired, and the color employed is of such a nature that it will dye vegetable and animal fibers, such as cotton, wool, silk, etc., and I employ a neutral vegetable oil soap, such as neutral cocoanut oil soap, for the reason that no free alkali is contained therein, as the animal fibers would not color well, should there be any free alkali. Moreover, the material is cleansed while the dyeing process is going on by using this neutral vegetable oil soap, as its scouring properties will not be affected perceptibly by a neutral product, such as sodium chlorid, which is subsequently added to force the dye on the vegetable and animal fiber. By reason of this combination of elements, the goods, either articles or material, when subjected to the action thereto, are thoroughly scoured and dyed in the same operation, the scouring being first accomplished, and the dyeing thereafter, by reason of the addition to the composition of the neutral product. Due to the softening qualities of the sulfonated castor oil, the goods, including buttonholes and seams, should they be a made-up garment, are softened and so permit the thorough cleansing and dyeing of the same.

The method of producing the detergent may be varied, but as an example, in a soap dye employing a black anilin color, I take

16 ozs. of neutral cocoanut oil soap, 2 ozs. of sulfonated castor oil, and one pint of water. This combination is boiled until the soap is thoroughly dissolved, and then I add three lbs. of anilin black dye, (substantive black), 60 which dyes both animal and vegetable fibers, such as cotton, wool, silk, etc., dissolved in one pint of water and which have been boiled together for a few minutes. The resultant mixture is boiled for a few minutes and then 65 poured into a mold to cool, and after hardening or solidifying, can be handled like ordinary cake soap.

The method or process of scouring and dyeing with the soap dye consists in subjecting the articles or materials to the action of the soap dye (consisting of neutral vegetable oil soap, sulfonated castor oil and anilin dye), dissolved in a boiling bath of water, and boil same for a suitable time, 75 such as five minutes. I then add a chemically neutral substance, such as sodium chlorid, which has the power to force the dye out of the boiling dye bath and onto both the animal and vegetable fibers at the 80 same time, and I boil slowly for a suitable time, say for fifteen or twenty minutes. The goods are then removed and washed in cold water. By adding the neutral product or neutral salt, which is neither acid nor alkali, 85 it will force the dye from the dye bath on all fibers, cotton, wool, silk, etc. (animal and vegetable fibers), and by first subjecting the goods to the soap dye, the same are thoroughly scoured or cleansed without the dye 90 taking any effect, so that the said dye bath will not stain to any extent the hands, nor the containers in which the goods are to be dyed, due to the fact that the soap keeps the dye from staining the same, but when the 95 neutral product, such as sodium chlorid, is added, the dye is taken up by the vegetable and animal fibers.

By this process, I obtain a color which is faster and brighter than if dyed in other 100 manners.

Having thus described my invention, what I claim as new and desire to secure by Letters Patent, is:

1. An alkali-free detergent for scouring 105 and dyeing, containing substantially in the proportions described, a neutral cocoanut oil soap, sulfonated castor oil, and anilin color adapted to dye both vegetable and animal fibers.

110

2. An alkali-free detergent for scouring and dyeing, containing, substantially in the proportions described, a neutral vegetable oil soap, sulfonated castor oil, and anilin 5 color adapted to dye both vegetable and animal fibers.
3. The process for producing a cake of dye-soap, consisting in boiling a neutral, vegetable oil soap, sulfonated castor oil and 10 water, substantially in the proportions de-

scribed, until dissolved, adding substantially in the proportion described, an anilin color adapted to dye both vegetable and animal fibers, dissolved in water, boiling this mixture, and then cooling it.

JOHN BARRINGTON.

Witnesses:

HARRY H. NOYES,  
JOHN P. MYRON.